

No. 661,650.

Patented Nov. 13, 1900.

S. H. THURSTON.

PROCESS OF COATING ONE METAL WITH ANOTHER AND RESULTING PRODUCT.

(Application filed Dec. 8, 1898.)

(Specimens.)



WITNESSES:

James F. Durham  
Charles W. Low

INVENTOR

Samuel Human Thurston  
BY  
James M. Hicks  
ATTORNEY

# UNITED STATES PATENT OFFICE.

SAMUEL H. THURSTON, OF LONG BRANCH, NEW JERSEY.

## PROCESS OF COATING ONE METAL WITH ANOTHER AND RESULTING PRODUCT.

SPECIFICATION forming part of Letters Patent No. 661,650, dated November 18, 1900.

Application filed December 8, 1898. Serial No. 698,670. (Specimens.)

*To all whom it may concern:*

Be it known that I, SAMUEL HEMAN THURSTON, a citizen of the United States of America, and a resident of Long Branch, county of Monmouth, State of New Jersey, have invented a certain new and useful Process of Coating One Metal with Another and the Products Resulting from Such Process, of which the following is a specification.

10 My invention relates to a process of coating one metal with another (especially iron and steel) with an amorphous, inherent, adherent, coherent permanent film or pellicle of one metal upon another, the particles of the coating metal being driven into and incorporated with the metal being coated by beating them into the interstices or pores at and beneath the surface thereof, as hereinafter specified; and it consists in a certain method of procedure fully set forth in this specification and claimed at the end thereof.

In previous applications, to which this present application is related, I have described and claimed the surfacing of iron and steel 25 with an amorphous, adherent, coherent, permanent coating of copper and copper oxide by a process similar in some respects to this present application.

To more fully specify the nature of the 30 process and the steps necessary to produce a more perfect and finished product is the object of this application, which steps are fully set out and claimed herein.

In order that persons skilled in the art to 35 which my invention appertains may understand, practice, and use my invention, I will proceed to describe it.

The first and a most important step consists in so cleaning the metal to be coated that 40 nothing remains upon its surfaces not homogeneous with the metal itself. Acids, alkalies, oxids, grease, and anything which prevents the coating metal from coming in absolute contact with the molecule of the metal to be 45 coated injures the result. The surfaces should be free from moisture, and preferably for the most perfect and permanent result the surfaces should be dried by heat. No air can remain between the molecules of the coating and the coated metal, and upon this depends the efficiency of the result. This is especially important where the metal to be

coated is an easily-oxidizable one, such as iron and steel, &c.

The second step in my process consists in impacting the coating metal into the surfaces to be coated by systematically beating the coating metal against the metal being coated, which is firmly held to receive the impacting blows of the beaters. This beating of the 55 coating metal upon the metal being coated is preferably produced by vibratory beating rods or pieces pivotally secured upon rods or supports on a rapidly-revolving drum located above a bed-plate arranged to move beneath 60 or over against the field of action of said beating-rods, on which bed-plate the metal plate being coated is firmly secured, so that by rapidly revolving said drum the beating-rods strike upon the surface of the metal on the 65 said bed-plate, and in doing so the metallic beating-rods first disturb the molecular condition of the said plate and serve to mechanically clean the surface, at the same time undoubtedly to open the pores of the said plate. 70 Then the particles from said beating-rods are hammered into the pores of the said plate and incorporated with its surface and form a pellicle of metal on its surface which is adherent to said surface and practically incorporated 75 with its particles or molecules and whose particles cohere with each other in such a manner that the said pellicle cannot be removed from said plate mechanically without removing the particles of the said plate also. 80

The manner of beating or driving the particles of coating metal into the pores of the metal being coated hereinbefore referred to is illustrated by the drawings herewith, in which— 85

Figure 1 represents a longitudinal view or elevation of a table for holding a plate of metal to be coated, driving-pulleys, and a cross-section on line  $x x$  of Fig. 2 of an apparatus in the nature of a wheel or flanges 95 provided with bars, on which are pivoted metal wires or beaters twisted about said bars and vibrating thereon. Fig. 2 is a front view of the table and a central section of the apparatus lengthwise of the apparatus for holding the vibratory wires or beaters, showing the end flanges, bearings, driving pulley-wheels, and beater-wires and rods which hold them. 100

A is the bed of the machine; B, the legs or supports.

C is the table on which the plate to be coated rests to be moved backward and forward either by hand or by the usual reciprocatory table movement, as in planing-machines, in which case the plate is fastened to the table; D, a raised portion of the table under the revolving vibrating beaters.

10 E is a shaft journaled in bearings F on the bed A at opposite sides of the bed.

G represents driving pulley-wheels secured on shaft E, by which the shaft E is driven in either direction circumferentially.

15 H represents flanges secured to shaft E, one at each end within the bearings F.

J represents rods which are secured to and in flanges E and extend from one flange to the other. On these rods J wires K are located, twisted about said rods so that they are free to swing on said bars.

L is the plate of metal to be coated. It rests on the bed C and is moved under the beating apparatus and on the curved raised portion D of the bed either by hand or by the forward movement of the table C, as the case may be. The revolution of the beating apparatus causes the wire beater K to strike with force upon the surface of the plate L, with more or less force as the distance from the surface of the plate is less or greater. This distance is regulated by turning the adjusting-box bearing-screws M in the usual manner, which raise or lower box-bearings N and of course raise or lower the shaft E, which is journaled therein. When an iron or steel plate L is being coated with copper, the wire beaters K are of copper in whole or in part. Of course the ends which beat upon the iron plate must in this case be copper. The result of this operation of my process by an apparatus is superior to the result produced by hand-beating; but my process is not confined to the use of an apparatus like the one herein described, but I prefer for regular surfaces to employ such an apparatus or its equivalent. Irregular surfaces are coated by my process either by hand-beating or by revolving beaters flexibly attached to and operated by mechanism driven by power, but manipulated by hand.

The results produced by this process are far superior to anything ever before produced by any previously-invented process and are permanent in their nature, and the coatings cannot be mechanically removed from the surfaces without removing the particles of the surface on which they are fixed. By this means the molecules of the coating are caused to forcibly adhere to the surfaces being coated and also to cohere between themselves. Thus an amorphous, permanent, inherent, adherent, coherent pellicle is formed upon the metal being coated, which may be rolled, extended, or bent without destroying the said film or pellicle. In performing this last step in my process the molecules of both coating and the

metal being coated are disturbed or disarranged and then rearranged, as the first effect of impacting or of impingement is to roughen the surfaces and disturb its molecules and at the same time to comminute the metal used in coating. It is also quite probable, as it is possible, that an electromagnetic condition is set up, especially in the case of copper when being impacted on iron and steel. I have found this condition in some cases to exist very strongly.

It is possible to rub one metal upon another and produce a color without much precaution other than ordinary cleaning and care; but such an operation does not in any manner resemble the process claimed by me as my discovery and invention, as the result is not permanent, adherent, or coherent and must be secured upon the surfaces by some binder, such as lacquer.

By this process I have succeeded in coating iron and steel with many metals and adapted it to a variety of cases and conditions, and in this application I shall claim such products as I deem important in a commercial point of view. These products are of an amorphous nature, not crystalline, as in the case of electrically-deposited and galvanized coatings previous to being burnished, which is an important difference and one which affects the usefulness of the coating produced by my invention.

By vigorously impacting one metal upon the other any particles which may have remained on the surfaces after the process or operation of cleaning are driven off and more thorough removal of deleterious matter occurs and a more perfect result is attained.

I am aware of the inventions and processes set out in the references, of record—viz., Dowling, British Patent No. 7,949 of 1839; Barron, British Patent No. 1,243 of 1856; Boucker, British Patent No. 12,720 of 1849; Potts, British Patent No. 2,764 of 1859; Spring, United States Patent No. 197,572, dated November 27, 1877; Bower, United States Patent No. 270,004, dated January 2, 1883; Elmore, British Patent No. 2,618, dated February 14, 1889, and I do not claim anything set out or claimed in said patents. None of them describes or claims any process which can possibly produce a product at all akin to that produced in accordance with my invention.

I claim—

1. The process substantially hereinbefore specified, which consists in producing a coating of one metal upon another, by first cleaning the metal to be coated substantially as specified, and then forcibly beating the coating metal upon the metal being coated systematically and continuously until the particles or molecules of the coating metal are driven into the pores of and incorporated with the particles at and beneath the surface of the metal being coated, and an amorphous inherent, adherent, coherent, permanent film or pellicle of the coating metal is formed upon

and irremovably united therewith, substantially as hereinbefore specified.

2. The within-described product consisting of a body of one metal whose surface particles are commingled with particles of another, coating metal, the coating metal being driven into the pores of the body metal, the two metals being incorporated together at and beneath the surface of the body metal, and forming a union the one with the other of a permanent nature, the one forming an in-

herent, adherent, amorphous, and coherent, coating upon the other, substantially as specified.

Signed by me at New York city, county and 15  
State of New York, this 1st day of December,  
1898.

SAMUEL H. THURSTON.

Witnesses:

JAMES M. HICKS,  
CHARLES W. LOW.